

1

3,038,797

### ALLOY STEEL FOR FORGINGS

Samuel J. Manganello, Wilkins Township, Allegheny County, and John E. Steiner, Churchill Borough, Pa., assignors to United States Steel Corporation, a corporation of New Jersey

No Drawing. Filed Nov. 13, 1959, Ser. No. 852,596  
4 Claims. (Cl. 75—128)

This invention relates to improvements in magnetic alloy steels for forgings and more particularly to alloy steels providing high yield strength combined with good notch toughness for large generator rotor forgings.

In the electric power industry, there is a need for a strong, tough, and magnetic steel suitable for large generator rotor forgings that serve as the rotating field components of large steam-turbine generators. These large rotor forgings range in diameter from 12 to 70 inches and in length from 15 to 35 feet. The steel rotors should be free of internal defects so they can withstand high operating stresses. They must be tough (nonbrittle) to resist the propagation of any internal or external cracks or defects present or incurred in service. Propagation of these cracks or defects results in sudden failure in service. In addition, these field rotor forgings should exhibit a high magnetic permeability (B/H or slope of the magnetization curve) to minimize the current necessary to generate the required magnetic field.

It is accordingly an object of this invention to provide alloy generator rotor forgings combining high yield strength, good notch toughness and high magnetic permeability.

It is another object to provide a readily forgeable alloy steel providing the foregoing properties.

The type of steel commonly used for rotor forgings for high speed generator units is a nickel, molybdenum, vanadium steel containing 0.18/0.33% carbon, 0.40/0.70% manganese, 0.15/0.40% silicon, 2.50% minimum nickel, 0.20/0.70% molybdenum, 0.03/0.12% vanadium, and sometimes up to 0.75% chromium if higher strength is desired. Such steel usually exhibits an 0.02% offset yield strength of about 65,000 to 90,000 p.s.i., a fracture appearance transition temperature (based on 50% shear fracture appearance) of 60 to 200° F., and a magnetizing force (H) of 600 to 1300 ampere-turns per inch to produce a flux density (B) of 130,000 lines per square inch. This steel falls far short of properties desired by the steam-turbine generator manufacturers for generator rotors, i.e. 90,000 p.s.i. yield strength (0.02% offset), 50° F. maximum fracture appearance transition temperature (50% shear), and 725 ampere-turns per inch,

2

met in a nickel, molybdenum, vanadium steel containing less than .40% manganese, between 3.50 and 4.25% nickel, and between .18 and .40% vanadium. Not only does such steel have an 0.02% offset yield strength in the range of 94,000 to 98,000 p.s.i. but such increase in yield strength is accompanied by a decrease in fracture appearance transition temperature to less than 50° F.

The fracture appearance transition temperature is determined by using V-notch Charpy specimens. The fracture appearance transition temperature differs from the more familiar ductility transition temperature. The fracture appearance transition temperature is determined by breaking specimens at different temperatures and determining from the appearance of the fractures at what temperature the steel failed in a 50%-ductile, 50%-brittle manner. Ductile fractures appear gray and fibrous, but brittle fractures appear silvery and granular; by comparing the fractured specimens with a chart, the relative ductility or brittleness of the fracture can readily be determined. In contrast, the ductility transition temperature is determined usually by measuring the energy absorbed in fracturing specimens at different temperatures and determining at what temperature the amount of energy absorbed suddenly increases or decreases. The fracture appearance transition temperature furnishes a more reliable and reproducible indication of the notch toughness of forging steels. Hereafter the term "transition temperature" will be used to indicate the fracture appearance transition temperature.

Our investigations have demonstrated that the desired properties may be obtained with the following components within the following ranges (percent by weight). It is preferable that rotor-forging ingots of the steel be vacuum cast.

| C    | Mn   | Si   | Ni   | Cr   | Mo   | V    | Al <sup>1</sup> |
|------|------|------|------|------|------|------|-----------------|
| 0.17 | 0.20 | 0.15 | 3.50 | 0    | 0.20 | 0.18 | max. 0.10       |
| 0.26 | 0.40 | 0.40 | 4.25 | 0.50 | 0.50 | 0.40 |                 |

Balance iron and usual impurities in common amounts.

<sup>1</sup> Acid-soluble.

The preferred range of components is as follows:

| C    | Mn   | Si   | Ni   | Cr   | Mo   | V    | Al <sup>1</sup> |
|------|------|------|------|------|------|------|-----------------|
| 0.18 | 0.20 | 0.15 | 3.70 | 0    | 0.20 | 0.18 | max. 0.05       |
| 0.24 | 0.35 | 0.40 | 4.00 | 0.30 | 0.30 | 0.30 |                 |

<sup>1</sup> Acid-soluble.

A typical composition of our new steel is:

| C    | Mn   | P     | S     | Si   | Ni   | Cr   | Mo   | V    | Al <sup>1</sup> | Fe                       |
|------|------|-------|-------|------|------|------|------|------|-----------------|--------------------------|
| 0.22 | 0.30 | 0.012 | 0.012 | 0.25 | 3.75 | 0.25 | 0.30 | 0.22 | 0.010           | Remainder and Impurities |

<sup>1</sup> Acid-soluble.

maximum, to produce a flux density of 130 kilolines per square inch.

We have discovered that the desired objectives can be

Test steels of the following compositions are illustrative of the unusual combination of properties resulting from the composition of our invention:

| Steel  | C    | Mn   | P     | S     | Si   | Ni   | Cr   | Mo   | V    | Al <sup>1</sup> |
|--------|------|------|-------|-------|------|------|------|------|------|-----------------|
| A----- | 0.19 | 0.32 | 0.011 | 0.015 | 0.32 | 2.97 | 0.28 | 0.26 | 0.09 | 0.045           |
| B----- | 0.17 | 0.31 | 0.012 | 0.013 | 0.24 | 3.65 | 0.27 | 0.32 | 0.10 | 0.054           |
| C----- | 0.21 | 0.30 | 0.009 | 0.013 | 0.24 | 2.97 | 0.26 | 0.28 | 0.22 | 0.006           |
| D----- | 0.22 | 0.31 | 0.010 | 0.013 | 0.23 | 3.72 | 0.28 | 0.31 | 0.22 | 0.069           |

<sup>1</sup> Acid-soluble.

Steel A is similar to the rotor forging steel mentioned hereinabove as being in common use in the industry; it differs from that rotor forging steel only in that it contains less manganese. Steel B is similar to Steel A except for a higher nickel content; Steel C is similar to Steel A with higher vanadium content. The results with these steels show that the desired properties cannot be obtained without increasing both nickel and vanadium. When both nickel and vanadium are increased the required amount and the manganese is low (Steel D), the desired properties are obtained.

Forged bars of these four steels were homogenized 2 hours at 1700° F., air cooled at room temperature, austenitized 4 hours at 1500° F., cooled at about 120° F. per hour to 600° F. (approximately the cooling rate that prevails at a location a few inches below the surface of a normalized 45-inch-diameter rotor forging), and free-furnace cooled to room temperature. This constitutes the normalizing treatment, to which all specimens were subjected. With air-cast steels, it is necessary to hold between 450 and 625° F. to prevent cracking or flaking. However our steel, if vacuum cast, may be air cooled to room temperature without harmful effects and in fact it has a beneficial effect on notch toughness without lowering the yield strength.

The tensile specimen blanks were tempered 24 hours at either 1140 or 1070° F. and air cooled. Tempering in the range of 1060 to 1080° F. is preferred. Tensile specimens (0.505-inch-diameter) were machined from the blanks and tested at room temperature. The following results were obtained:

Table I

| Steel | Temper-<br>ing<br>Temp.,<br>° F. | Yield Point,<br>p.s.i. |        | Yield Strength,<br>p.s.i. |                | Tensile<br>Strength,<br>p.s.i. | Elongation<br>in 2",<br>Percent | Reduction<br>of Area,<br>Percent |
|-------|----------------------------------|------------------------|--------|---------------------------|----------------|--------------------------------|---------------------------------|----------------------------------|
|       |                                  | Upper                  | Lower  | 0.02%<br>Offset           | 0.2%<br>Offset |                                |                                 |                                  |
| A     | 1,140                            | 80,500                 | 79,600 | 80,400                    | 79,700         | 98,200                         | 24.5                            | 66.0                             |
| A     | 1,070                            | -----                  | -----  | 80,400                    | 82,000         | 103,400                        | 24.5                            | 64.0                             |
| B     | 1,140                            | -----                  | -----  | 88,750                    | 92,950         | 109,000                        | 19.5                            | 64.4                             |
| B     | 1,070                            | -----                  | -----  | 92,350                    | 98,700         | 115,300                        | 22.0                            | 65.9                             |
| C     | 1,140                            | 79,000                 | 74,400 | 79,000                    | 74,600         | 90,300                         | 27.5                            | 67.6                             |
| D     | 1,140                            | 94,700                 | 89,600 | 93,700                    | 89,800         | 104,200                        | 24.5                            | 67.2                             |
| D     | 1,070                            | 97,800                 | 96,400 | 97,800                    | 96,400         | 112,500                        | 23.0                            | 65.7                             |

After normalizing, the impact-specimen blanks were tempered 24 hours at either 1140 or 1070° F., then either brine-quenched or slowly cooled (about 7° F. per hour to 750° F., then free-furnace cooled to room temperature). Charpy V-notch impact specimens were then machined from the blanks and tested at temperatures in the range -100° F. to +80° F. The following results were obtained:

Table II

| Steel | Temper-<br>ing<br>Temp., ° F. | Transition Temp., ° F.                     |                                              |
|-------|-------------------------------|--------------------------------------------|----------------------------------------------|
|       |                               | Slowly<br>Cooled<br>From<br>Temper-<br>ing | Brine-<br>Quenched<br>From<br>Temper-<br>ing |
| A     | 1,140                         | 50                                         | 35                                           |
| A     | 1,070                         | 60                                         | 35                                           |
| B     | 1,140                         | 75                                         | 55                                           |
| B     | 1,070                         | 60                                         | 55                                           |
| C     | 1,140                         | 10                                         | -10                                          |
| D     | 1,140                         | -20                                        | -40                                          |
| D     | 1,070                         | 0                                          | -20                                          |

After normalizing, some of the magnetic-test specimen blanks were tempered for 24 hours at 1160° F., free-furnace cooled, tempered 24 hours at 1120° F., and again free-furnace cooled (both coolings at about 150° F. per hour). Other magnetic-test specimen blanks were tempered at 1070° F. and were similarly cooled. Magnetic-test specimens (1 1/16 inches wide by 1/4 inch thick by 12 inches long) were machined from the tempered blanks

and tested at room temperature. The following results were obtained:

| Steel | Ampere-Turns per<br>Inch for 130 Kilolines<br>per Square Inch |                          |
|-------|---------------------------------------------------------------|--------------------------|
|       | 1,160° F. +<br>1,120° F.                                      | 1,110° F. +<br>1,070° F. |
| A     | 747                                                           | -----                    |
| B     | 626                                                           | -----                    |
| C     | 788                                                           | 718                      |
| D     | 727                                                           | 707                      |

After normalizing and tempering, the steels of our invention have a microstructure consisting essentially of ferrite and bainite.

The results given above show that the desired 0.02% offset yield strength (90,000 p.s.i.) is not obtained in Steel A but is obtained in Steel B tempered at 1070° F. Furthermore, the magnetic properties of Steel B are very good (magnetizing force of 626 ampere-turns per inch). However, the transition temperature of Steel B, though good, is still rather high (60° to 75° F.). By increasing the vanadium content from 0.10 to 0.22%, however, a marked improvement in the transition temperature was obtained (Steels C and D). Steel C, which contains only 2.97% nickel, exhibits a low transition temperature (10° F.) but also exhibits a low yield strength (79,000 p.s.i.) like Steel A. This indicates that 2.97% nickel or 0.22% vanadium, by itself, will not give an 0.02%

offset yield strength of 90,000 p.s.i.

By increasing the nickel content from 2.97% to above 3.50% and the vanadium content to above .18%, however, the desired combination of high strength, good notch toughness, and high magnetic permeability (relatively low magnetizing force value) was obtained (Steel D). Moreover, Steel D was only slightly susceptible to temper embrittlement, as shown by the increase of only 20° F. in the transition temperature of the specimens slowly cooled from tempering over the transition temperature of those brine-quenched from tempering. It is believed that the low manganese content of Steel D contributed greatly toward its relative insensitivity to temper embrittlement.

The mechanisms by which increases in nickel and, to a lesser degree, vanadium improve the strength of the nickel, molybdenum, vanadium steel are not fully understood, but it is believed that nickel strengthens the ferrite and that vanadium forms carbides that also serve to strengthen the steel. Vanadium, above about 0.18%, improves the notch toughness of nickel, molybdenum, vanadium steel by one or more of the following mechanisms:

- (1) Refining the austenitic and ferritic grain size. (The austenite grain size of the steels containing 0.22% vanadium was ASTM No. 7 or finer, and the ferrite grain size was 8 1/2 or finer. An austenite grain size of ASTM No. 4 or finer is desirable, as such fineness of grain is necessary for satisfactory ultrasonic testing.)
- (2) Combining with and hence lowering the amount of carbon in solution.

(3) Decreasing, perhaps, the susceptibility of nickel, molybdenum, vanadium steel to temper embrittlement.

The low manganese content is believed to make the steel less susceptible to temper embrittlement.

This application is a continuation-in-part of our co-pending application Serial No. 803,829, filed April 3, 1959, now abandoned.

While we have shown and described several specific embodiments of our invention, it will be understood that these embodiments are merely for the purpose of illustration and description and that various other forms may be devised within the scope of our invention, as defined in the appended claims.

We claim:

1. A steel characterized by an 0.02% offset yield strength in excess of 90,000 p.s.i., a transition temperature below 50° F., a high magnetic permeability, as indicated by a magnetizing force of below 725 ampere-turns per inch to produce a flux density of 130 kilolines per square inch and substantial freedom from temper embrittlement, said steel containing by weight

.17 to .26% carbon  
.20 to .40% manganese  
.15 to .40% silicon  
3.50 to 4.25% nickel  
.20 to .50% molybdenum  
.18 to .40% vanadium  
Up to .50% chromium  
.10% max. acid soluble aluminum

balance iron and residual impurities.

2. A generator rotor forging characterized by an 0.02% offset yield strength in excess of 90,000 p.s.i., a transition temperature below 50° F., a high magnetic permeability, as indicated by a magnetizing force of below 725 ampere-turns per inch to produce a flux density of 130 kilolines per square inch, a ferritic-bainitic microstructure and substantial freedom from temper embrittlement, said steel containing by weight

.17 to .26% carbon  
.20 to .40% manganese  
.15 to .40% silicon  
3.50 to 4.25% nickel  
.20 to .50% molybdenum  
.18 to .40% vanadium  
Up to .50% chromium  
.10% max. acid soluble aluminum

balance iron and residual impurities.

3. A steel characterized by an 0.02% offset yield strength in excess of 90,000 p.s.i., a transition temperature below 50° F., a high magnetic permeability, as indicated by a magnetizing force of below 725 ampere-turns per inch to produce a flux density of 130 kilolines per square inch and substantial freedom from temper embrittlement, said steel containing by weight

.18 to .24% carbon  
.20 to .35% manganese  
.15 to .40% silicon  
3.70 to 4.00% nickel  
Up to .30% chromium  
.20 to .30% molybdenum  
.18 to .30% vanadium  
.05% max. acid soluble aluminum

balance iron and residual impurities.

4. A generator rotor forging characterized by an 0.02% offset yield strength in excess of 90,000 p.s.i., a transition temperature below 50° F., a high magnetic permeability, as indicated by a magnetizing force of below 725 ampere-turns per inch to produce a flux density of 130 kilolines per square inch, a ferritic-bainitic microstructure and substantial freedom from temper embrittlement, said steel containing by weight

.18 to .24% carbon  
.20 to .35% manganese  
.15 to .40% silicon  
3.70 to 4.00% nickel  
Up to .30% chromium  
.20 to .30% molybdenum  
.18 to .30% vanadium  
.05% max. acid soluble aluminum

balance iron and residual impurities.

#### References Cited in the file of this patent

#### UNITED STATES PATENTS

|    |           |                 |                |
|----|-----------|-----------------|----------------|
| 40 | 934,697   | Schneider       | Sept. 21, 1909 |
|    | 1,261,742 | Churchward      | Apr. 2, 1918   |
|    | 2,206,370 | Scherer         | July 2, 1940   |
| 45 | 2,845,345 | Bauscher et al. | July 29, 1958  |

#### OTHER REFERENCES

Hall: Nickel in Iron and Steel, 1954, page 168. Published by John Wiley and Sons, Inc., New York, N.Y.